

## UNITED STATES PATENT OFFICE

2,065,929

## PRIMING COMPOSITION

Alfred Weale, Heswall, England, assignor, by  
mesne assignments, to Remington Arms Com-  
pany, Inc., Bridgeport, Conn., a corporation of  
Delaware

No Drawing. Application September 9, 1931,  
Serial No. 561,994. In Great Britain Septem-  
ber 19, 1930

## 4 Claims. (Cl. 102—18)

This invention relates to improved priming compositions for propellant cartridges, and it comprises priming compositions for percussion caps adapted for propellant cartridges, said 5 priming composition comprising lead azide, guanylnitrosaminoguanyl tetrazene and barium nitrate, as an oxidizing agent, and advantageously also comprising a fuel such as calcium silicide, and having improved properties includ- 10 ing increased sensitiveness rendering them advantageous for use in percussion caps.

It has already been proposed to employ lead azide as an ingredient of percussion cap compositions, but its application has been limited. 15 Against its use it has been urged that lead azide is dangerous to manufacture, has a low sensitiveness, and that compositions containing it are too violent in action: the addition of other ingredients customary in percussion cap manu- 20 facture, while slightly decreasing the violence of action, has a further deleterious effect upon the sensitiveness. The use of colloidal lead azide in place of the crystalline variety, whilst increasing safety in manufacture, results in a still less 25 sensitive composition.

The advantages accruing from the use of the lead azide are as follows:—

(1) Increased safety in manufacturing operations due to the low sensitiveness of the uncom- 30 pressed compositions, which do not bear any exact relation in sensitiveness to compositions as finally compressed in the cap shell.

(2) Economy, due firstly to the low cost of lead azide and the large proportions of cheap 35 ingredients which may be used, and secondly to the low charge of the composition itself.

(3) The great stability of lead azide compositions.

(4) By replacing mercury fulminate, season 40 cracking of the brass cartridge cases is eliminated.

I have discovered means by which priming compositions containing lead azide may be prepared so as to obtain all the normal advantages 45 of its use while eliminating certain defects and disadvantages heretofore considered more or less fundamental and inherent in the use of lead azide.

I have now found that compositions contain- 50 ing lead azide both of the colloidal and crystalline varieties can be made to conform to specifications of sensitiveness by the inclusion of guanylnitrosaminoguanyl tetrazene, in the mix. The violence of such compositions can be 55 regulated as desired by the addition of fuels and

oxidizing agents in suitable proportions without the deleterious effect upon the sensitiveness previously mentioned.

A priming composition adapted for percussion caps made in accordance with my present invention, comprises lead azide, guanylnitrosaminoguanyl tetrazene, barium nitrate (as an oxidizing agent) and, advantageously, a fuel such as calcium silicide. 5

When the lead azide content is low, for ex- 10 ample between 5% and 10% of the total mix, and the content of the other, and more inert, ingredients consequently high, a large proportion of guanylnitrosaminoguanyl tetrazene, for example from 10% to 15% of the total mix, 15 should be added to bring the sensitiveness of the final mix to the required level. If, on the other hand, the lead azide content is higher, for example between 15% and 20% of the total mix, a smaller proportion of tetrazene, for ex- 20 ample from 0.5% to 5% of the total mix, is sufficient to sensitize the final mix.

The sensitivity of a cap composition depends partly on the hardness of the ingredients, and I find that in compositions that do not contain 25 much hard material it is sometimes necessary to use a higher proportion of guanylnitrosaminoguanyl tetrazene together with a high proportion of lead azide.

Compositions containing lead azide and the 30 higher proportions of guanylnitrosaminoguanyl tetrazene have the great advantage over those containing low proportions of guanylnitrosaminoguanyl tetrazene of binding well and not breaking away under the pressing punches. 35

Typical cap compositions which may be used are the following:—

|                                   | Per cent | Per cent |
|-----------------------------------|----------|----------|
| Lead azide                        | 25.0     | 14.0     |
| Barium nitrate                    | 54.5     | 46.0     |
| Calcium silicide                  | 20.0     | 20.0     |
| Guanylnitrosaminoguanyl tetrazene | 0.5      | 10.0     |
| Lead peroxide                     | —        | 10.0     |

During the manufacture of these compositions, the lead azide, especially the colloidal variety, 45 tends to separate out from the other ingredients during the loading of the caps. This does not occur if the lead azide content is increased to about 50%, but, as has been stated such a high content is undesirable as the caps are too violent. An efficient percussion cap is obtained if the composition is loaded in two layers. A layer of composition rich in lead azide is first introduced, and then a layer consisting of a fuel, such as calcium silicide, and an oxidizing agent 55

such as barium nitrate, only. Such a cap contains a low total content of lead azide and functions through the lower layer exploding and disintegrating the upper layer. The fuel and oxidizing agent in this layer, being in the form of an extremely fine powder and very intimately mixed, produce a large flame.

Typical compositions for use in this manner are:—

|    |                                   |         |
|----|-----------------------------------|---------|
| 10 | (1) Layer in base of cap shell    | Percent |
|    | Lead azide                        | 35      |
|    | Barium nitrate                    | 60      |
| 15 | Guanylnitrosaminoguanyl tetrazene | 5       |
|    | (2) Upper layer                   |         |
|    | Barium nitrate                    | 50      |
|    | Calcium silicide                  | 50      |

I do not restrict myself to any particular ingredients other than lead azide and guanylnitrosaminoguanyl tetrazene or to any particular method of mixing the ingredients.

There is a difference between American and British usage of the term "cap." In the present specification by the term "cap" I mean caps adapted for priming cartridges, that is, propellant cartridges, and I do not intend to include detonators for explosive shells, bombs or blasting explosives, in such terms.

I claim:—

1. An improved percussion cap comprising a loading of an improved priming composition containing 15% to 20% of lead azide and 0.5% to 5% of guanylnitrosaminoguanyl tetrazene, said loading comprising two contiguous loads, one of which comprises the lead azide and the guanylnitrosaminoguanyl tetrazene and the other contiguous load comprising calcium silicide and barium nitrate.

2. A primer for the ignition of the propellant powder of a small arms cartridge comprising a mixture of lead azide and guanylnitrosaminoguanyl tetrazene, and contiguous thereto a second mixture of calcium silicide and barium nitrate.

3. A primer for the ignition of the propellant powder of a small arms cartridge comprising a mixture of lead azide, guanylnitrosaminoguanyl tetrazene and barium nitrate, and contiguous thereto a second mixture of calcium silicide and barium nitrate.

4. A primer for the ignition of the propellant powder of a small arms cartridge comprising a mixture of approximately 35% of lead azide, 5% of guanylnitrosaminoguanyl tetrazene, and 60% of barium nitrate; and contiguous thereto a second mixture of approximately 50% of calcium silicide and 50% of barium nitrate.

ALFRED WEALE. 30